# EUROPEAN PATENT SPECIFICATION

(11) **EP 1 526 215 B1**
(45) Date of publication and mention of the grant of the patent: **09.09.2009**
(21) Application number: 04022942.9
(22) Date of filing: 27.09.2004
(51) Int. Cl.: D06N 3/00, D06N 7/00, D06M 15/564, D06M 15/263

(54) **Layered product based on non-woven fabric, particularly for exposed trims, and method for manufacturing the product**
Beschichteter Vliesstoff, insbesondere für Innenbekleidung von Kraftfahrzeugen, und Verfahren zu dessen Herstellung
Non-tissé revêtu, notamment pour la garniture intérieure de véhicules automobiles, et son procédé de fabrication

(30) Priority: 24.10.2003 IT PD20030260
(43) Date of publication of application: 27.04.2005
(73) Proprietor: O.R.V. OVATTIFICIO RESINATURA VALPADANA S.p.A., 35010 Grantorto (Padova) (IT)
(72) Inventor: Peruzzo, Maurizio, 36061 Bassano del Grappa (Vicenza) (IT)
(74) Representative: Modiano, Micaela Nadia

(56) References cited:
- EP-A- 0 296 701
- WO-A-03/004759
- DE-A1- 2 029 517
- US-A- 3 713 868

## Description

The present invention relates to a layered product based on non-woven fabric.

The product is used particularly but not exclusively for exposed trims in the field of motor vehicles or of vehicles in general, as an internal lining for the cabin roof.

Applications in the field of furniture and clothing, for example, are also foreseeable.

The invention also relates to the method for manufacturing the layered product.

It is known that the internal lining of the roof of the cabin of cars or vehicles in general is composed of a soft padding designed to act as a barrier, generally made of at least one web of non-woven fabric, and of an exposed fabric lining, such as a jersey or a Malivlies fabric, for outward appearance.

This structure arises because it is currently impossible to provide a non-woven fabric that can be used, on its own, for exposed trims.

The non-woven fabric that is used, in view of its nature (polyester and/or polyamide fibers) and of its technical and structural characteristics, is in fact currently unable to pass the tests normally used by car manufacturers for resistance to abrasion, safety and light-fastness (the product degrades over time due to solar radiation).

Fabrics coated with resins of the type defined in the precharacterizing portion of the appended claim 1 are described in the documents WO 03/004759 A, EP-A-0 296 701, and DE 20 29 517 A1.

The aim of the present invention is to provide a layered product based on non-woven fabric that can be used as is for exposed trims, accordingly without the need to combine it, outside of its production cycle, with covering elements.

Within this aim, an object of the present invention is to provide a layered product based on non-woven fabric that allows a manufacturing simplification of exposed trims and a cost reduction.

Another object is to provide a layered product based on non-woven fabric that allows higher flexibility of the production process to obtain a finished product having the most disparate appearances.

Another object is to provide a layered product based on non-woven fabric that can be manufactured with a method that is advantageous in terms of hourly productivity.

Another object is to provide a layered product based on non-woven fabric that can be manufactured without particular technological complications with respect to known products.

Another object is to provide a layered product based on non-woven fabric whose cost for raw materials is not higher than that of current products.

Another object is to provide a layered product based on non-woven fabric that can be manufactured by using current facilities.

In accordance with the invention, there is provided a layered product based on non-woven fabric, as defined in the appended claims 1-7.

Advantageously, the method for manufacturing said layered product of the appended claims 1-7 is defined in the appended claims 8-9.

Further characteristics and advantages of the present invention will become better apparent from the following detailed description of a preferred but not exclusive embodiment thereof, and of its production method, illustrated by way of non-limiting example in the accompanying drawings, wherein:
Figure 1 is a view of a first embodiment of an apparatus for producing the layered product according to the invention;
Figure 2 is a view of a second embodiment of an apparatus for producing the layered product according to the invention;
Figure 3 is a view of a third embodiment of an apparatus for producing the layered product according to the invention.

With reference to Figure 1, a layered product based on non-woven fabric according to the invention comprises at least one web 10 of non-woven fabric and at least one layer 11 of a mixture based on foamable resin that is resistant to abrasion, soft and light-fast, and covers at least one of the two sides of the at least one web 10 of non-woven fabric.

Preference is given to a plurality of webs of hydroentangled non-woven fabric (hydroentanglement is designed to make the basic substrate more uniform and therefore more suitable for the end result) and a mixture based on resin, selected in a group comprising polyurethane- and/or acrylic-based resins.

In particular, the composition of the non-woven fabric can be for example selected advantageously among the following (% by weight):
-- 100% polyester
-- 70% polyester, 30% polyamide
-- 50% polyester, 50% polyamide

As regards the resin mixture, it can be conveniently for example (% by weight):
-- cross-linking acrylic resin 57.4%
-- cross-linking agent 0.7%
-- expanding agent 7.0%
-- stabilizing fillers 10.5%
-- color 7.0%
-- thickening agents 3.4%
-- deionized water 14.0%

Also by way of example, the finished product can be constituted by:
-- 120-140 g/m² of non-woven fabric
-- 30-40 g/m² of resin-based mixture
-- final thickness: 1-1.2 mm
-- final grammage: 150-180 g/m²

The method for producing such layered product based on non-woven fabric consists of a preliminary step for producing the hydroentangled non-woven fabric by using oven temperatures of approximately 60-80 °C, lower than the background art, and by keeping the stretching during fiber carding at low levels in order to achieve very high longitudinal elongations, and in then applying the resin-based mixture on the surface of at least one side.

The required elongations are:

| | |
|---|---|
| at 20 N, in a longitudinal direction | 2.2 - 3.5% |
| at 20 N, in a transverse direction | 6.5 - 11% |
| at 50 N, in a longitudinal direction | 9.0 - 15% |
| at 50 N, in a transverse direction | 20-27% |
| at 100 N, in a longitudinal direction | 20-27% |
| at 100 N, in a transverse direction | 32-38% |

The method of application of the resin-based mixture is such that it does not stress the material and at the same time is capable of distributing a very low quantity of resin absolutely uniformly, for example 30 to 40 g/m², as already mentioned, it avoids losing the particular characteristics of the non-woven fabric (strengths, elongations, et cetera), and finally allows said resin to remain on the surface as much as possible.

The preferred method is the application of foamed resin by means of a rotating cylinder, as described hereinafter.

Figure 1 is a diagram of an apparatus, generally designated by the reference numeral 12, for depositing the layer of foamed resin 11 on the web 10.

The apparatus 12 comprises a rotating cylinder 13, for example such as the one manufactured by the Stork company, which is combined with a foaming unit, designated by the reference numeral 14, of which only a component described hereinafter is shown.

The rotating cylinder 13 is hollow, with through holes 13a formed uniformly on the wall, and is provided internally with a device 15 for distributing the foam (designated by the reference numeral 15a) on the wall of the cylinder 13.

The device 15, of a per se known type, is termed "squeegee" and is part of the foaming unit 14.

The foaming unit 14 has a very important role, since the density of the foam directly influences the quantity of resin deposited on the material.

Once the foam of the chosen density has been obtained, it passes within the squeegee 15, which is provided with a spreading blade 16; the blade 16 can have different lengths and can therefore give flexibility to the dosage system. It is also possible to adjust the inclination angle and the pressure applied by the blade 16 to the cylinder 13.

In practice, for each foam density, by acting on the adjustments of the squeegee it is possible to distribute uniformly different quantities of resin, ranging from 5 to 120 g/m².

The apparatus 12 further has an additional blade 17 for adjusting the thickness of the layer of resin 11, which is external with respect to the rotating cylinder 13 and arranged downstream thereof.

The additional adjustment blade 17 provides adjustment of the thickness once the resin has been deposited by the cylinder 13 on the web 10.

The system for moving the web 10 is provided by conveyor rollers 18 that are arranged opposite the rotating cylinder 13.

In practice, the web 10 passes through the sort of calender formed by the conveyor rollers 18 and by the rotating cylinder 13.

Respective washing devices 19, of a per se known type, for the web 10 are associated with the rollers 18.

Figure 2 illustrates a diagram of a second embodiment of the apparatus for depositing said layer of foamed resin on at least one hydroentangled web; said apparatus is now designated by the reference numeral 112.

In this embodiment, the squeegee device 115 arranged inside the cylinder 113 is inclined with respect to the first embodiment of Figure 1, so as to indicate the possibility to provide embodiments of the apparatus that have mutually different inclinations of the exit of the resin 111, in order to optimize the step for distributing said resin on the at least one hydroentangled web 110.

Figure 3 illustrates a diagram of a third embodiment of the apparatus for depositing said layer of foamed resin on at least one hydroentangled web; said apparatus is now designated by the reference numeral 212.

In this embodiment there are two rotating cylinders 213 in series containing a squeegee 215, so as to obtain a different flexibility on the control of the thickness of the layer of resin and on the number of layers.

In practice it has been found that the present invention has achieved the intended aim and objects.

The layered product based on non-woven fabric described above can in fact be used as is for exposed trims, without therefore having to be combined, outside of its production cycle, with covering fabrics, saving their corresponding costs.

The layered product allows a manufacturing simplification of exposed trims and a cost reduction, and also allows higher flexibility of the manufacturing process in order to obtain a finished product that has the most disparate appearances, for example by means of successive printing operations performed on the exposed surface.

As the skilled in the art would understand, all the technical details may further be replaced with other technically equivalent elements.

The materials, so long as they are compatible with the contingent use, as well as the dimensions, may be any according to requirements, without thereby abandoning the scope of the protection of the appended claims.

Where technical features mentioned in any claim are followed by reference signs, those reference signs have been included for the sole purpose of increasing the intelligibility of the claims and accordingly such reference signs do not have any limiting effect on the interpretation of each element identified by way of example by such reference signs.

## Claims

1. A layered product based on non-woven fabric, comprising:
-- at least one web of hydroentangled non-woven fabric (10, 110);
-- at least one layer (11, 111) of a foamed resin-based mixture that is resistant to abrasion, soft and light-fast, and covers at least one of the two sides of said at least one web of non-woven fabric;
the layered product being **characterized in that** it is constituted by:
-- 120-140 g/m² of non-woven fabric (10, 110); and
-- 30-40 g/m² of foamed resin-based mixture (11, 111).

2. The layered product based on non-woven fabric according to claim 1, **characterized in that** said at least one web of non-woven fabric (10, 110) is 100% polyester.

3. The layered product based on non-woven fabric according to claim 1, **characterized in that** said at least one web of non-woven fabric (10, 110) is 70% polyester and 30% polyamide.

4. The layered product based on non-woven fabric according to claim 1, **characterized in that** said at least one web of non-woven fabric (10, 110) is 50% polyester and 50% polyamide.

5. The layered product based on non-woven fabric according to one of the preceding claims, **characterized in that** said resin of said foamed resin-based mixture is selected in a group comprising polyurethane- and/or acrylic-based resins.

6. The layered product based on non-woven fabric according to claims 1 or 5, **characterized in that** said foamed resin-based mixture is composed of:
-- cross-linking acrylic resin 57.4%;
-- cross-linking agent 0.7%;
-- expanding agent 7.0%;
-- stabilizing fillers 10.5%;
-- color 7.0%;
-- thickening agents 3.4%;
-- deionized water 14.0%, and
by weight.

7. The layered product based on non-woven fabric of claim 1, wherein the layered product has a thickness of 1-1.2 mm, and a weight of 150-180 g/m².

8. A method for producing a layered product based on non-woven fabric according to one or more of the preceding claims, consisting in applying at the surface, on at least one side of an intermediate component composed of at least one web of 120-140 g/m² of non-woven fabric (10, 110) a mixture based on resins selected in a group comprising foamed, abrasion-resistant, soft and light-fast polyurethane- and/or acrylic-based resins so as to provide 30-40 g/m² of resin (11, 111) in the layered product

9. The method according to claim 8, which consists in applying foamed resin by means of at least one rotating cylinder (13, 113, 213), which is hollow with through holes (13a) on its wall and is provided internally with a device (15, 115, 215) for distributing the foamed resin of the "squeegee" type.

## Patentansprüche

1. Lagenprodukt auf Vliesstoffbasis, mit:
- zumindest einer Bahn aus wasserstrahlverfestigtem Vliesstoff (10, 110);
- zumindest einer Schicht (11, 111) aus einer geschäumten Mischung auf Harzbasis, die abriebresistent, weich und lichtecht ist und zumindest eine der beiden Seiten der zumindest einen Vliesstoff-Bahn bedeckt;
wobei das Lagenprodukt **dadurch gekennzeichnet ist, dass** es aus:
- 120 bis 140 g/m² Vliesstoff (10, 110); und
- 30 bis 40 g/m² geschäumter Mischung (11, 111) auf Harzbasis besteht.

2. Lagenprodukt auf Vliesstoffbasis nach Anspruch 1, **dadurch gekennzeichnet, dass** die zumindest eine Bahn aus Vliesstoff (10, 110) 100 % Polyester ist.

3. Lagenprodukt auf Vliesstoffbasis nach Anspruch 1, **dadurch gekennzeichnet, dass** die zumindest eine Bahn aus Vliesstoff (10, 110) 70 % Polyester und 30 % Polyamid ist.

4. Lagenprodukt auf Vliesstoffbasis nach Anspruch 1, **dadurch gekennzeichnet, dass** die zumindest eine Bahn aus Vliesstoff (10, 110) 50 % Polyester und 50 % Polyamid ist.

5. Lagenprodukt, auf Vliesstoffbasis nach einem der vorherigen Ansprüche, **dadurch gekennzeichnet, dass** das Harz der geschäumten Mischung auf Harzbasis aus einer Gruppe umfassend Harze auf Polyurethan- und/oder Akrylbasis ausgewählt ist.

6. Lagenprodukt auf Vliesstoffbasis nach Anspruch 1 oder 5, **dadurch gekennzeichnet, dass** die geschäumte Mischung auf Harzbasis aus:
- vernetzendem Akrylharz, 57,4 Gew.-%;
- Vernetzungsmittel, 0,7 Gew.-%;
- Treibmittel, 7,0 Gew.-%;
- stabilisierenden Füllstoffen, 10,5 Gew.-%;
- Farbstoff, 7,0 Gew.-%;
- Dickungsmitteln, 3,4 Gew.-%; und
- entionisiertem Wasser, 14,0 Gew.-%
zusammengesetzt ist.

7. Lagenprodukt auf Vliesstoffbasis nach Anspruch 1, wobei das Lagenprodukt eine Dicke von 1 bis 1,2 mm und ein Gewicht von 150 bis 180 g/m² aufweist.

8. Verfahren zum Herstellen eines Lagenprodukts auf Vliesstoffbasis nach einem oder mehreren der vorherigen Ansprüche, bestehend aus dem Auftragen einer Mischung auf die Oberfläche zumindest einer Seite einer Zwischenkomponente, die aus zumindest einer Bahn aus 120 bis 140 g/m² Vliesstoff (10, 110) besteht, wobei die Mischung auf Harzen basiert, die aus der Gruppe umfassend geschäumte, abriebresistente, weiche und lichtechte Harze auf Polyurethan- und/oder Akrylbasis ausgewählt sind, um 30 bis 40 g/m² Harz (11, 111) im Lagenprodukt bereitzustellen.

9. Verfahren nach Anspruch 8, welches im Auftragen von geschäumtem Harz mittels zumindest eines Drehzylinders (13, 113, 213) besteht, der hohl ist und in seiner Wand Durchgangslöcher (13a) aufweist und im Inneren mit einer Vorrichtung (15, 115, 215) in der Art eines "Quetschers" zum Verteilen des geschäumten Harzes versehen ist.

## Revendications

1. Produit stratifié à base de tissu non tissé, comprenant :
- au moins une nappe de tissu non-tissé (10, 110) hydro-emmêlé,
- au moins une couche (11, 111) d'un mélange moussé à base de résine qui résiste à l'abrasion, doux et résistant à la lumière, qui couvre au moins l'un des deux côtés de la ou des nappes de tissu non tissé, le produit stratifié étant **caractérisé en ce qu'**il est constitué de :
- 120 à 140 g/m² de tissu non tissé (10, 110) et
- 30 à 40 g/m² du mélange moussé (11, 111) à base de résine.

2. Produit stratifié à base du tissu non tissé selon la revendication 1, **caractérisé en ce que** ladite ou lesdites nappes de tissu non tissé (10, 110) sont constituées de 100 % de polyester.

3. Produit stratifié à base d'un tissu non tissé selon la revendication 1, **caractérisé en ce que** ladite ou lesdites nappes de tissu non tissé (10, 110) sont constituées de 70 % de polyester et de 30 % de polyamide.

4. Produit stratifié à base d'un tissu non tissé selon la revendication 1, **caractérisé en ce que** ladite ou lesdites nappes de tissu non tissé (10, 110) sont constituées de 50 % de polyester et de 50 de polyamide.

5. Produit stratifié à base de tissu non tissé selon l'une des revendications précédentes, **caractérisé en ce que** ladite résine dudit mélange moussé à base de résigne est sélectionnée dans l'ensemble constitué des résines à base de polyuréthane et/ou d'acrylique.

6. Produit stratifié à base de tissu non tissé selon les revendications 1 ou 5, **caractérisé en ce que** ledit mélange moussé à base de résine est constitué de :
- 57,4 % de résine acrylique apte à réticuler,
- 0,7 % d'agent de réticulation,
- 7,0 % d'agent de gonflement,
- 10,5 % de charges de stabilisation,
- 7,0 % de colorant,
- 3,4 % d'agents épaississants, et
- 14,0 % d'eau déminéralisée,
les pourcentages étant en poids.

7. Produit stratifié à base de tissu non tissé selon la revendication 1, dans lequel le produit stratifié présente une épaisseur de 1 à 1,2 mm et un poids par unité de surface de 150 à 180 g/m².

8. Procédé de production d'un produit stratifié à base de ti.ssu non tissé selon une ou plusieurs des revendications précédentes, consistant à appliquer à la surface d'au moins un côté d'un composant intermédiaire constitué d'au moins une nappe de 120 à 140 g/m² de tissu non tissé (10, 110) un mélange à base de résines sélectionnées dans l'ensemble constitué des résines à base de polyuréthane et/ou d'acrylique, moussé, résistant à l'abrasion, doux et résistant à la lumière, de manière à doter le produit stratifié de 30 à 40 g/m² de résine (11, 111).

9. Procédé selon la revendication 8, qui consiste à appliquer une résine moussée au moyen d'au moins un cylindre rotatif (13, 113, 213) creux dont la paroi est traversée par des trous (13a) et dont l'intérieur est doté d'un dispositif (15, 115, 215) de répartition de la résine moussée de type raclette.
